



US010933464B2

(12) **United States Patent**  
**Wu**

(10) **Patent No.:** **US 10,933,464 B2**  
(45) **Date of Patent:** **Mar. 2, 2021**

(54) **FORGING CAST METHOD USING THIN SHELL MOLD**

(71) Applicant: **Cheng-Kuan Wu**, Tainan (TW)

(72) Inventor: **Cheng-Kuan Wu**, Tainan (TW)

(\*) Notice: Subject to any disclaimer, the term of this patent is extended or adjusted under 35 U.S.C. 154(b) by 0 days.

(21) Appl. No.: **16/519,477**

(22) Filed: **Jul. 23, 2019**

(65) **Prior Publication Data**

US 2021/0023612 A1 Jan. 28, 2021

(51) **Int. Cl.**

**B22D 18/04** (2006.01)  
**B22D 18/06** (2006.01)  
**B22C 9/04** (2006.01)  
**B22D 18/02** (2006.01)  
**B22C 9/03** (2006.01)

(52) **U.S. Cl.**

CPC ..... **B22D 18/02** (2013.01); **B22C 9/03** (2013.01); **B22C 9/04** (2013.01); **B22D 18/04** (2013.01); **B22D 18/06** (2013.01)

(58) **Field of Classification Search**

CPC ..... B22D 18/04; B22D 18/06; B22D 27/13; B22C 9/04

See application file for complete search history.

(56)

**References Cited**

**U.S. PATENT DOCUMENTS**

5,299,619 A \* 4/1994 Chandley ..... B22D 27/04  
164/133  
6,932,145 B2 \* 8/2005 Frasier ..... B22C 9/02  
164/122.2  
2003/0024681 A1 \* 2/2003 Soderstrom ..... B22C 9/08  
164/122.1  
2017/0312813 A1 \* 11/2017 Wu ..... B22C 9/12

**FOREIGN PATENT DOCUMENTS**

GB 2454010 A \* 4/2009 ..... B22D 27/15

\* cited by examiner

*Primary Examiner* — Kevin E Yoon

(74) *Attorney, Agent, or Firm* — Alan D. Kamrath; Karin L. Williams; Mayer & Williams PC

(57) **ABSTRACT**

A casting method includes preparing a thin shell mold which is sintered and placed in a box. Sands are buried in the box to encompass the thin shell mold. The pressure chamber is depressurized. The casting material is filled into the thin shell mold, such that the thin shell mold is disposed at a vacuum state. Then, the negative pressure of the pressure chamber is released. Then, the pressure chamber is pressurized, to form a pressure difference which presses the casting material to flow into the thin shell mold, thereby finishing the casting work. The temperature of the casting material is reduced, and the pressure in the pressure chamber is increased. Then, the casting material is cooled to form a casting product. Then, the thin shell mold is broken, and the casting product is removed.

**5 Claims, 10 Drawing Sheets**





F I G . 1



F I G . 2



F I G . 3



FIG. 4



FIG. 5



FIG. 6



FIG. 7



FIG. 8



FIG. 9



FIG. 10

## 1

## FORGING CAST METHOD USING THIN SHELL MOLD

## BACKGROUND OF THE INVENTION

## 1. Field of the Invention

The present invention relates to a molding method of a metallic mold and, more particularly, to a forging cast (or squeeze casting) method using a thin shell mold.

## 2. Description of the Related Art

A conventional casting process comprises gravity casting and low pressure casting. In the gravity casting, a metal is melted and poured into a casting die. Then, the melted metal is solidified to form a casting product. Thus, the gravity casting is worked simply to save the cost. However, the gravity casting wastes material. In addition, air is introduced during the casting process, thereby decreasing the quality of the product. In the low pressure casting, liquid casting material is filled into a die, to perform a casting work under a negative pressure. Thus, the casting work is performed under the negative pressure, to prevent from introducing the air, such that the casting product has a clean surface. A ceramic mold is formed by a dewaxing method and has a fine surface. However, the ceramic mold has a complicated working process. In addition, the ceramic mold cannot tolerate a high pressure. A forging cast (or squeeze casting) method comprises filling a melted metal into a mold, applying a high pressure before the melted metal is solidified, such that the melted metal is solidified under the high pressure. Thus, the casting product formed by the forging cast method has a precise size, and will not produce cracks during the casting process. However, the forging cast method is only available for a mold with greater thickness and strength to withstand the high pressure. In addition, the mold the forging cast method has an expensive price. Further, the metal mold dissipates the heat quickly, such that the inner face and the outer face of the casting product are not cooled evenly.

## BRIEF SUMMARY OF THE INVENTION

The primary objective of the present invention is to provide a forging cast method using a thin shell mold, wherein the casting material is filled and casted in the thin shell mold by a pressure differential, and is cooled under a positive pressure to form the casting product, thereby preventing the thin shell mold from being broken when subjected to the pressure.

In accordance with the present invention, there is provided a casting method comprising a first step of preparing a mold, a second step of sintering, a third step of depressurizing, a fourth step of filling, a fifth step of pressurizing, a sixth step of molding, and a seventh step of finishing work. The first step includes preparing a thin shell mold and a pressure chamber. The thin shell mold is made of ceramic material and has a thickness of 0.5-2.0 mm. The thin shell mold has an upper end provided with a sprue having a diameter of 25-45 mm. The thin shell mold has a periphery provided with a plurality of support brackets. The thin shell mold has a smooth inner surface and a rough outer surface. The pressure chamber has an interior provided with a furnace and a box. The furnace is provided with a feeding device. The box is provided with a temperature control device. The second step includes sintering the thin shell

## 2

mold at a temperature under 600° C. The third step includes placing the thin shell mold in the box, then burying sands in the box to encompass and support the thin shell mold, then depressurizing and keeping a negative pressure in the pressure chamber at a value of -0.002 MPA to -0.05 MPA, and then turning on the temperature control device to heat the box under the negative pressure of the pressure chamber. The sands closely compress the thin shell mold and the support brackets. The rough outer surface of the thin shell mold touches the sands to increase a contact area between the thin shell mold and the sands. The fourth step includes melting casting material in the furnace of the pressure chamber under the negative pressure of the pressure chamber, and then filling the casting material through the feeding device of the furnace and the sprue of the thin shell mold into the thin shell mold. The feeding device of the furnace squeezes the casting material at a pressure of 10-20 KG/cm<sup>2</sup> to cover the sprue of the thin shell mold. The casting material is filled into the sprue of the thin shell mold to isolate an inner space of the thin shell mold from the pressure chamber, such that the inner space of the thin shell mold is disposed at a vacuum state. The fifth step includes stopping filling the casting material, then releasing the negative pressure of the pressure chamber, then introducing air into the pressure chamber to pressurize the pressure chamber, then forming a pressure difference between the inner space of the thin shell mold and the pressure chamber to press the casting material to further flow into the inner space of the thin shell mold, and then finishing a casting work after the casting material stops flowing. The sixth step includes turning off the temperature control device to reduce the temperature of the casting material in the thin shell mold, then increasing the pressure in the pressure chamber to a positive value of 80-100 KG/cm<sup>2</sup>, to squeeze the casting material in the thin shell mold, and then cooling the casting material to form a casting product. The casting material is forced by the pressure of the pressure chamber to press an inner wall of the thin shell mold, and the sands in the box are forced by the pressure of the pressure chamber to press an outer wall of the thin shell mold. The casting material closely press the inner wall of the thin shell mold, such that the casting product has a smooth and clean surface. The seventh step includes removing the thin shell mold from the box, then breaking the thin shell mold, and then removing the casting product from the thin shell mold.

Further benefits and advantages of the present invention will become apparent after a careful reading of the detailed description with appropriate reference to the accompanying drawings.

## BRIEF DESCRIPTION OF THE SEVERAL VIEWS OF THE DRAWING(S)

FIG. 1 is a flow chart of a casting method in accordance with the preferred embodiment of the present invention.

FIG. 2 is a flow chart of steps S1 to S4 of the casting method in accordance with the preferred embodiment of the present invention.

FIG. 3 is a flow chart of steps S5 to S7 of the casting method in accordance with the preferred embodiment of the present invention.

FIG. 4 is a cross-sectional view of a thin shell mold in accordance with the preferred embodiment of the present invention.

FIG. 5 is a cross-sectional operational view showing the pressure chamber is depressurized in accordance with the preferred embodiment of the present invention.

FIG. 6 is a cross-sectional operational view showing the cover is pressed in accordance with the preferred embodiment of the present invention.

FIG. 7 is a cross-sectional operational view showing the casting material is filled and pressed in accordance with the preferred embodiment of the present invention.

FIG. 8 is a cross-sectional operational view showing the pressure chamber is pressurized in accordance with the preferred embodiment of the present invention.

FIG. 9 is a locally enlarged cross-sectional operational view showing a pressurizing state in accordance with the preferred embodiment of the present invention.

FIG. 10 is another locally enlarged cross-sectional operational view showing a pressurizing state in accordance with the preferred embodiment of the present invention.

#### DETAILED DESCRIPTION OF THE INVENTION

Referring to FIGS. 1-10, a casting method in accordance with the preferred embodiment of the present invention comprises a first step S1 of preparing a mold, a second step S2 of sintering, a third step S3 of depressurizing, a fourth step S4 of filling, a fifth step S5 of pressurizing, a sixth step S6 of molding (or forming or shaping), and a seventh step S7 of finishing work.

The first step S1 includes preparing a thin shell mold 1 (see FIG. 4) and a pressure chamber 2 (see FIG. 5). The thin shell mold 1 is made of ceramic material and has a thickness of 0.5-2.0 mm. The thin shell mold 1 has an upper end provided with a sprue (or gate) 11 having a diameter of 25-45 mm. The thin shell mold 1 has a periphery provided with a plurality of support brackets 12 which are arranged in a vertical direction. The thin shell mold 1 has a smooth inner surface and a rough outer surface. A dilute slurry is poured into the thin shell mold 1, with a surplus slurry being introduced outward from the thin shell mold 1. Thus, the smooth inner surface is formed in the thin shell mold 1 after the slurry is dried. The pressure chamber 2 has an interior provided with a furnace 21 and a box 3. The furnace 21 is provided with a feeding device 211. The box 3 is provided with a temperature control device 31 to control the temperature in the box 3.

The second step S2 includes sintering (or agglomerating) the thin shell mold 1 at a temperature under 600° C. The sintering process strengthens the thin shell mold 1 to withstand thermal expansion and contraction, thereby preventing the thin shell mold 1 from being broken due to the thermal expansion and contraction. The thin shell mold 1 is sintered at a low temperature, to prevent vitrification.

As shown in FIG. 5, the third step S3 includes placing the thin shell mold 1 in the box 3, then burying sands 30 in the box 3 to encompass and support the thin shell mold 1, then depressurizing and keeping a negative pressure in the pressure chamber 2 at a value of -0.002 MPa to -0.05 MPa, and then turning on the temperature control device 31 to heat the box 3 under the negative pressure of the pressure chamber 2. The sands 30 closely compress the thin shell mold 1 and the support brackets 12. The rough outer surface of the thin shell mold 1 touches the sands 30 to increase a contact area between the thin shell mold 1 and the sands 30. The sands 30 and the rough outer surface of the thin shell mold 1 conduct and distribute a heat to the thin shell mold 1 evenly to enhance the heat conduction.

As shown in FIG. 7, the fourth step S4 includes melting casting material in the furnace 21 of the pressure chamber 2 under the negative pressure of the pressure chamber 2, and

then filling the casting material through the feeding device 211 of the furnace 21 and the sprue 11 of the thin shell mold 1 into the thin shell mold 1. The feeding device 211 of the furnace 21 squeezes and fills the casting material at a pressure of 10-20 KG/cm<sup>2</sup> to cover the sprue 11 of the thin shell mold 1 by the casting material. The casting material is filled into the sprue 11 of the thin shell mold 1 to isolate an inner space of the thin shell mold 1 from the pressure chamber 2, such that the inner space of the thin shell mold 1 is disposed at a vacuum state.

As shown in FIG. 8, the fifth step S5 includes stopping filling the casting material, then removing the feeding device 211 of the furnace 21 from the sprue 11 of the thin shell mold 1, then releasing the negative pressure of the pressure chamber 2, then introducing air into the pressure chamber 2 to pressurize the pressure chamber 2, then forming a pressure difference between the inner space of the thin shell mold 1 and the pressure chamber 2 to press the casting material to further flow into the inner space of the thin shell mold 1, and then finishing a casting work after the casting material stops flowing.

Referring to FIG. 9 with reference to FIG. 8, the sixth step S6 includes turning off the temperature control device 31 to reduce the temperature of the casting material in the thin shell mold 1, then increasing the pressure in the pressure chamber 2 to a positive value of 80-100 KG/cm<sup>2</sup>, to squeeze the casting material in the thin shell mold 1, and then cooling the casting material to form a casting product 4 as shown in FIG. 10. The casting material is forced by the pressure of the pressure chamber 2 to press an inner wall of the thin shell mold 1, and the sands 30 in the box 3 are forced by the pressure of the pressure chamber 2 to press an outer wall of the thin shell mold 1 as shown in FIG. 9, such that the thin shell mold 1 is compressed between the casting material and the sands 30 to form a pressure balance, thereby preventing the thin shell mold 1 from being damaged due to a pressure difference. The casting material closely press the inner wall of the thin shell mold 1, such that the casting product 4 has a smooth and clean surface.

The seventh step S7 includes removing the thin shell mold 1 from the box 3, then breaking the thin shell mold 1, and then removing the casting product 4 from the thin shell mold 1.

In the fourth step S4, the casting material in the furnace 21 of the pressure chamber 2 is disposed at a semisolid state. The fifth step S5 further includes successively heating the casting material in the thin shell mold 1 by the temperature control device 31 during a period of 2-7 minutes after the casting work is finished, and then increasing the pressure in the pressure chamber 2 to 25-30 KG/cm<sup>2</sup>, such that the thin shell mold 1 and the casting material are combined closely. In the sixth step S6, when the casting material is cooled, a contraction rate of the casting material is reduced.

In the first step S1, the box 3 has an upper end provided with a cover 32 which has a through hole 321 allowing passage of the sprue 11 of the thin shell mold 1.

The fifth step S5 further includes applying a pressure of 5-15 KG/cm<sup>2</sup> on the cover 32 as shown in FIG. 6, and then forcing the sands 30 to apply a pressure on the thin shell mold 1 evenly. As shown in FIG. 7, the casting material is filled into the sprue 11 of the thin shell mold 1 under the pressurized condition.

In the fifth step S5, when the air is introduced into the pressure chamber 2, the pressure in the pressure chamber 2 exceeds the atmospheric pressure and is kept at 15-50 KG/cm<sup>2</sup>, during a period of 2-5 minutes, such that the casting material in the sprue 11 of the thin shell mold 1 is

subjected to the pressure in the pressure chamber 2 to fill the inner space of the thin shell mold 1, and the thin shell mold 1 is heated successively.

It is appreciated that, the thin shell mold 1 is made of ceramic material that is not available for a high pressure working condition of a forging cast (or squeeze casting) process. In the present invention, the inside of the thin shell mold 1 presents a negative pressure, and the outside of the thin shell mold 1 presents a positive pressure, such that the thin shell mold 1 made of ceramic material can be used in the forging cast process by using the pressure differential of the thin shell mold 1. Thus, the thin shell mold 1 has a small thickness to save the cost of material.

In fabrication, the thin shell mold 1 is formed by a dewaxing method or by a 3-D printing machine. The thin shell mold 1 has a thickness of 0.5-2.0 mm to save the ceramic material. The sprue 11 of the thin shell mold 1 has a diameter of 25-45 mm to reduce a hydraulic jump action during the casting process, thereby preventing the casting product 4 from being damaged. The support brackets 12 support the thin shell mold 1 and will not obstruct the heating effect. The thin shell mold 1 has a smooth inner surface such that the casting product 4 has a smooth surface. Then, the thin shell mold 1 is sintered such that the thin shell mold 1 withstands a high pressure. In addition, the thin shell mold 1 is sintered at a low temperature, such that the thin shell mold 1 withstands a temperature differential. Then, the sands 30 are buried into the box 3, to encompass and support the outside of the thin shell mold 1. Then, the pressure chamber 2 is depressurized and kept at the negative pressure of -0.002 MPa to -0.05 MPa. Then, the temperature control device 31 heats the box 3 under the negative pressure, such that the sands 30 conduct and transmit the heat to the thin shell mold 1 evenly. The thin shell mold 1 has a small thickness, such that the heat is distributed on the thin shell mold 1 quickly, to perform a preheat process. Then, the casting material is heated and melted. Then, the casting material is filled through the sprue 11 into the thin shell mold 1, and the feeding device 211 of the furnace 21 pressurizes the casting material at a pressure of 10-20 KG/cm<sup>2</sup> to fill the casting material into the thin shell mold 1. At this time, the sands 30 and the support brackets 12 support the thin shell mold 1 to counteract the force applied by the casting material. Then, the casting material is filled with and covers the sprue 11 of the thin shell mold 1 to isolate the inner space of the thin shell mold 1 from the pressure chamber 2, such that the unfilled inner space of the thin shell mold 1 is disposed at a vacuum state. Then, the air is introduced into the pressure chamber 2 such that the pressure chamber 2 is returned to the atmospheric pressure. Thus, a pressure differential is defined between the outside and the inside of the thin shell mold 1 such that the casting material is filled into the thin shell mold 1 to fill the inner space of the thin shell mold 1. Then, the temperature control device 31 is turned off to reduce the temperature of the casting material in the thin shell mold 1. Then, the pressure in the pressure chamber 2 is increased to 80-100 KG/cm<sup>2</sup>, such that the casting material is cooled under a high pressure to form the casting product 4. Then, the thin shell mold 1 is broken, and the casting product 4 is removed from the thin shell mold 1.

Accordingly, the thin shell mold 1 is compressed between the casting material and the sands 30 to form a pressure balance, thereby preventing the thin shell mold 1 from being damaged due to a pressure difference. In addition, the casting material closely press the inner wall of the thin shell mold 1, such that the casting product 4 has a smooth and clean surface. Further, the casting material is filled and

casted in the thin shell mold 1 by a pressure differential, and is cooled under a positive pressure to form the casting product 4, thereby preventing the thin shell mold 1 from being broken when subjected to the pressure. Further, the thin shell mold 1 has a small thickness to save the cost of material.

In experiment, the present invention provides testing data as follows.

The casting material is disposed at a liquid state and is not fully filled with the thin shell mold 1, the pressure chamber 2 is under a negative pressure of -0.05 MPa, and an inert gas is introduced into the pressure chamber 2 to increase the pressure in the pressure chamber 2. The pressure resistant capacity of the thin shell mold 1 corresponds to the thickness of the thin shell mold 1 and the applied pressure, and the table of the thickness versus pressure of the thin shell mold 1 is listed as follows.

| thickness | pressure              |                       |                       |                       |                       |
|-----------|-----------------------|-----------------------|-----------------------|-----------------------|-----------------------|
|           | 15 kg/cm <sup>2</sup> | 20 kg/cm <sup>2</sup> | 30 kg/cm <sup>2</sup> | 40 kg/cm <sup>2</sup> | 50 kg/cm <sup>2</sup> |
| 0.5 mm    | ○                     | ○                     | ○                     | X                     | X                     |
| 1.0 mm    | ○                     | ○                     | ○                     | X                     | X                     |
| 1.5 mm    | ○                     | ○                     | ○                     | ○                     | X                     |
| 2.0 mm    | ○                     | ○                     | ○                     | ○                     | ○                     |
| 2.5 mm    | ○                     | ○                     | ○                     | ○                     | ○                     |

It is clear that, when the casting material is not fully filled with the thin shell mold 1, the pressure resistant capacity of the thin shell mold 1 is reduced if the thickness of the thin shell mold 1 is decreased. For example, when the thin shell mold 1 with a thickness of 0.5 mm is subjected to a pressure greater than 40 KG/cm<sup>2</sup>, the thin shell mold 1 cannot tolerate the low pressure and will be broken. Thus, when the casting material is not fully filled with the thin shell mold 1, it is necessary to reduce the pressure and to keep the preheat state.

After the casting material is fully filled with the thin shell mold 1, the outside and the inside of the thin shell mold 1 reaches a pressure balance, so that the thin shell mold 1 can withstand a higher pressure, and the table of the thickness versus pressure of the thin shell mold 1 is listed as follows.

| thickness | pressure              |                       |                       |                       |                        |
|-----------|-----------------------|-----------------------|-----------------------|-----------------------|------------------------|
|           | 80 kg/cm <sup>2</sup> | 85 kg/cm <sup>2</sup> | 90 kg/cm <sup>2</sup> | 95 kg/cm <sup>2</sup> | 100 kg/cm <sup>2</sup> |
| 0.5 mm    | ○                     | ○                     | ○                     | ○                     | ○                      |
| 1.0 mm    | ○                     | ○                     | ○                     | ○                     | ○                      |
| 1.5 mm    | ○                     | ○                     | ○                     | ○                     | ○                      |
| 2.0 mm    | ○                     | ○                     | ○                     | ○                     | ○                      |
| 2.5 mm    | ○                     | ○                     | ○                     | ○                     | ○                      |

It is clear that, when the casting material is fully filled with the thin shell mold 1, the thin shell mold 1 with a thickness of 0.5 mm can withstand a high pressure of 100 KG/cm<sup>2</sup>, such that the thickness of the thin shell mold 1 is reduced to save the cost of material. It is appreciated that, when the thickness of the thin shell mold 1 is decreased, the heat radiation efficiency is increased.

Alternatively, when the casting material is heated to a semisolid metallic state (such as paste) and filled into the thin shell mold 1, the table of the thickness versus pressure of the thin shell mold 1 is listed as follows.

| thickness | pressure                 |                          |                          |                          |                          |
|-----------|--------------------------|--------------------------|--------------------------|--------------------------|--------------------------|
|           | 15<br>kg/cm <sup>2</sup> | 20<br>kg/cm <sup>2</sup> | 30<br>kg/cm <sup>2</sup> | 40<br>kg/cm <sup>2</sup> | 50<br>kg/cm <sup>2</sup> |
| 0.5 mm    | X                        | ○                        | ○                        | ○                        | X                        |
| 1.0 mm    | X                        | ○                        | ○                        | ○                        | X                        |
| 1.5 mm    | X                        | ○                        | ○                        | ○                        | ○                        |
| 2.0 mm    | X                        | ○                        | ○                        | ○                        | ○                        |
| 2.5 mm    | X                        | ○                        | ○                        | ○                        | ○                        |

5 10 15 20 25 30 35 40 45 50

It is clear that, the semisolid metal has a low fluidity, such that it is necessary to apply a higher pressure to squeeze the casting material when the casting material is disposed at the semisolid metallic state. However, the semisolid metal has a low deformation, such that the thin shell mold 1 with a smaller thickness can tolerate a higher pressure. In addition, the semisolid metal has a temperature lower than that of the liquid metal, such that the semisolid metal has a smaller contraction when being cooled, to obtain the casting product 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10000 10005 10010 10015 10020 10025 10030 10035 10040 10045 10050 10055 10060 10065 10070 10075 10080 10085 10090 10095 10100 10105 10110 10115 10120 10125 10130 10135 10140 10145 10150 10155 10160 10165 10170 10175 10180 10185 10190 10195 10200 10205 10210 10215 10220 10225 10230 10235 10240 10245 10250 10255 10260 10265 10270 10275 10280 10285 10290 10295 10300 10305 10310 10315 10320 10325 10330 10335 10340 10345 10350 10355 10360 10365 10370 10375 10380 10385 10390 10395 10400 10405 10410 10415 10420 10425 10430 10435 10440 10445 10450 10455 10460 10465 10470 10475 10480 10485 10490 10495 10500 10505 10510 10515 10520 10525

mold is subjected to the pressure in the pressure chamber to fill the inner space of the thin shell mold, and the thin shell mold is heated successively.

\* \* \* \* \*